

Aug. 1, 1967

J. MALLEN ET AL  
PROCESS FOR THE MANUFACTURE OF PRODUCTS OF BERYLLIUM  
OR BERYLLIUM ALLOY  
Filed Oct. 6, 1964

3,333,994



## 1

3,333,994

 PROCESS FOR THE MANUFACTURE OF  
PRODUCTS OF BERYLLIUM OR BERYL-  
LIUM ALLOY

José Mallen, Paris and Michel Weisz, Orsay, France, as  
signors to Commissariat à l'Energie Atomique, Paris,  
France

Filed Oct. 6, 1964, Ser. No. 401,862

 Claims priority, application France, Oct. 25, 1963,  
951,895

7 Claims, (Cl. 148—11.5)

The present invention relates to improvements in processes for the manufacture of beryllium products which are intended notably for aviation, aeronautics and atomic energy.

It concerns more particularly processes of this type which are concerned with the production of beryllium tubes, and more particularly tubes suitable for the casting of fuel elements of nuclear reactors.

Since the beginning of the utilisation of beryllium in aircraft and then in space craft, and finally as a nuclear material, for which fields it is particularly suitable by virtue of its remarkable physical properties, the desired beryllium products have always been made from billets or blooms of sintered beryllium. Only some parts of simple shape, such as sheets, have been obtainable from cast metal, and even then it has been necessary to effect a grain refinement in order that this material may have acceptable mechanical characteristics.

Endeavours have therefore been made to improve the ductility of beryllium tubes and for this reason recourse has hitherto been had to powder metallurgy for the production of such tubes, since the sintered metal has a much finer grain than the cast metal, as also much higher longitudinal ductility (in the direction of the cold working at low temperature).

However, despite many efforts to increase the three-dimensional ductility, tubes of this type have proved incapable of meeting certain requirements in regard to casings for nuclear fuels.

Of the many stresses which are set up in the course of the operation of the reactor, the casing of a fuel "pencil," i.e. of a rod of very small diameter in relation to its length, must notably withstand with an appropriate safety margin those which correspond to the thermal stresses resulting from its association with the fuel (each of these members has its own programme temperature and its own coefficient of expansion).

During continuous operation, the casing is at a temperature which is determined by its position, the neutron balance of the reactor, the speed of the cooling fluid, etc., and it is normally sufficiently hot to afford relief from any stresses.

In transient operation, particularly during cooling, the situation is more critical owing to the thermal stresses set up in the casing. In this respect, the entry temperature of the fluid, usually 200–250° C., is of great importance.

It has been found that with a casing, the major problem is to obtain sufficient transverse ductility at low temperature in order to avoid rupture.

Tubes obtained by powder metallurgy do not possess such ductility in a sufficient degree. Efforts have therefore been directed to the production of tubes possessing this essential form of ductility and it has been discovered that, to some extent, the longitudinal ductility and the grain size are only of secondary importance.

The present invention therefore has the object of providing a process for the preparation of products of beryllium or beryllium alloy and particularly tubes, which more fully satisfies than hitherto the various practical re-

## 2

quirements, and in particular permits of obtaining a less fragile product of more favourable texture which is not detrimentally affected by maintenance for long periods at temperatures of the order of 700° C., which is much cleaner from the viewpoint of inclusions, exhibits few intergranular flaws and above all possesses distinctly higher transverse ductility.

The invention resides mainly in that—while an ingot of cast beryllium or beryllium alloy, optionally subjected to a compression, is used as starting material—the said ingot is subjected, in the course of its shaping to at least one cold working operation, optionally followed by a tepid drawing, a straightening by stress relief with imparted deformation at a temperature close to that of the recrystallisation of the metal, and followed by a controlled recrystallisation annealing.

The invention further comprises, apart from this main feature, certain other features which are preferably used at the same time, and which are to be considered separately or in any technically possible combinations:

The said cold working operation or operations consist in impact extrusion, the metal being optionally coated with a thin layer of silver,

The said cold working operation or operations consist in extrusion under a casing, which casing may notably consist of soft steel,

The said cold working operation or operations consist in a pre-extrusion under a thin casing followed by an extrusion under a thick casing,

The extent of the extrusion is at least equal to 50.

In any case, the invention will be more readily understood from the following further description and the following example, which are, of course, given only by way of example. In the course of this description, reference will be made to the single figure which gives, as a function of temperature, the transverse ductility of the beryllium treated by the process according to the invention and of sintered beryllium.

The use of cast metal as starting material, instead of sintered metal as usual, is one of the most important features of the present invention because it shows that cold-worked cast metal is substantially free from hot fragility, that its texture is more favourable than that of cold-worked sintered metal, that maintenance at 600–700° C. for long periods is beneficial to the cold-worked cast metal, while it is harmful to cold-worked sintered metal, that inclusion radiographs have revealed higher "cleanliness" of the cold-worked cast metal, and finally that, although its presentation and its surface appearance seem to be less good, it is less subject to defects such as intergranular microcracks, which are harmful to transverse ductility in the case of tubes.

The following table shows a comparison of the longitudinal and transverse ductilities of sintered and cast beryllium ingots:

|                             | Minimum temperature for an elongation of 10% |                       |
|-----------------------------|----------------------------------------------|-----------------------|
|                             | Longitudinal (DL), ° C.                      | Transverse (DT), ° C. |
| Extruded sintered sheet bar | 50                                           | >400                  |
| Extruded cast sheet bar     | 140                                          | 250                   |

Since the transverse ductility is much higher than the longitudinal ductility in the case of tubes, notably those intended for casing, the superiority of cast beryllium will be apparent from this table.

After the choice of cast metal in preference to sintered metal, the choice of the cold working operation becomes a factor of second order. Methods as different as impact

extrusion or the conventional extrusion under a casing may be used, but the second method gives greater lengths of more uniform tubes, as will hereinafter be seen with reference to the following example.

The tubes of cold-worked cast metal according to the present invention may also be subjected to a tepid drawing which improves the tolerances of the surface condition, and gives greater pliability in the controlled recrystallisation treatments. Thus, drawing passes of 10 to 15% at 450° C. are possible without intermediate annealing.

The tubes thus prepared are thereafter subjected to stress relief followed by annealing at a temperature close to the recrystallisation temperature, i.e. between 550° and 750° C., which process improves the elastic limit at elevated temperature and the ductility of the beryllium.

There will therefore be given in the following an example of the production of beryllium tubes by the process according to the present invention.

There is used as starting material a cast beryllium ingot which is compressed for 2 minutes at 650° C. under a pressure of 10,000 bars, this compression having the object of eliminating any remaining small pores and thus providing a "clean" ingot.

In the course of a pre-extrusion at 950° C., a billet in the form of a thin soft steel casing 2 mm. thick is cold-worked to a degree or an area reduction of 6.

The bar thus obtained is cut into sections and pierced to supply the billets intended for the extrusion of tubes.

A second extrusion is thereafter performed at 950° C. at a speed of 27 mm./second and to a cold-working degree or an area reduction of 15.

The trueing of the tubes is thereafter effected by deformation imparted in tension, in the course of which a considerable stress relief occurs at 650° C. in half an hour, and annealed at 750° C. for 4 hours. As stated in the foregoing, the product obtained is more ductile and less fragile than an equivalent product prepared from sintered metal, as is shown by comparison of the curves A and B of the single figure.

Curve A corresponds to a beryllium tube obtained by the process of the invention. Curve B corresponds to a sintered tube. "Dr%" is the percentage of elongation at the moment of rupture of a test bar subject to traction.

Of course, the invention is in no way limited to the mode of application just referred to, or to the embodiment described, but covers all variants thereof, and notably the manufacture of all beryllium products from cast metal,

not only for nuclear uses, but also for requirements of aviation and aeronautics.

What is claimed is:

1. A method for manufacturing tubes of beryllium and beryllium alloy comprising the steps of first working a cast ingot of beryllium and beryllium alloy at about 950° C. with an area reduction of about 6, then further working said ingot at about 950° C. with an area of reduction of about 15, then subjecting the drawn ingot to stress relief with plastic deformation in tension at a temperature approaching recrystallization temperature of the metal in the range of 550-750° C. and then annealing at a temperature of about 750° C. for about four hours.

15 2. A method as described in claim 1, including the step of first compressing the cast ingot of beryllium and beryllium alloy at about 650° C.

3. A method as described in claim 1, including the step, after the further working step, of then tepid drawing said ingot at about 450° C.

10 4. A method as described in claim 1, said working steps comprising impact extrusion, the ingot being coated with a thin layer of silver.

5. A method as described in claim 1, said working steps consisting of extrusion under a casing of soft steel.

6. A method as described in claim 1, said first working step consisting of extrusion under a thin casing followed by said further working step of extrusion step under a thick casing.

15 7. A method as described in claim 1, said working steps consisting of hot extrusion of the ingot with an area reduction at least equal to 50:1.

#### References Cited

##### UNITED STATES PATENTS

|           |         |              |       |          |
|-----------|---------|--------------|-------|----------|
| 2,872,363 | 2/1959  | Macherey     | ----- | 148—11.5 |
| 3,065,117 | 11/1962 | Brown et al. | ----- | 148—13   |
| 3,234,052 | 2/1966  | Wikle        | ----- | 148—11.5 |

##### FOREIGN PATENTS

|         |         |                |
|---------|---------|----------------|
| 868,064 | 5/1961  | Great Britain. |
| 884,108 | 12/1961 | Great Britain. |
| 884,410 | 12/1961 | Great Britain. |
| 919,423 | 2/1963  | Great Britain. |

40 45 DAVID L. RECK, Primary Examiner.

H. F. SAITO, Assistant Examiner.